

1,374,277.

R. H. BROWNLEE.  
LUBRICATING OIL.  
APPLICATION FILED NOV. 23, 1918.

Patented Apr. 12, 1921.



# UNITED STATES PATENT OFFICE.

ROY H. BROWNLEE, OF PITTSBURGH, PENNSYLVANIA.

## LUBRICATING-OIL.

1,374,277.

Specification of Letters Patent. Patented Apr. 12, 1921.

Original application filed May 13, 1918, Serial No. 234,077. Divided and this application filed November 23, 1918. Serial No. 263,829.

To all whom it may concern:

Be it known that I, Roy H. BROWNLEE, a citizen of the United States, residing at Pittsburgh, in the county of Allegheny and State of Pennsylvania, have invented certain new and useful Improvements in Lubricating-Oils, of which the following is a specification.

My invention relates to an improved lubricating oil of low specific gravity, low cold test, and high viscosity, having the properties of lubricating oils made from the finest asphaltic base crudes, from hydrocarbons of petroleum distillates.

15 In making my improved oil, I may utilize any suitable hydrocarbon made from the lighter vaporous and condensed products of hydrocarbon oils, but prefer the product of the process of treating hydrocarbon oils 20 forming the subject matter of my prior application, filed March 29, 1917, Serial No. 158,165. The lubricating oil of the present application is the product of the process or method forming the subject matter of my 25 prior application filed May 13, 1918, series No. 234,077, of which the subject matter of the present application is a division.

The desired product results from treating a petroleum distillate containing a considerable percentage of unsaturated hydrocarbons within an inclosed vessel in the presence of a suitable catalyst, capable of polymerizing the unsaturated hydrocarbons at a suitable temperature with accompanying 35 agitation, to effect the desired reaction and separation of useful vapors from other undesirable products. Thereafter, the agitation is temporarily discontinued, the accumulated sludge is drawn off, and a small portion of the lighter vapors may be distilled off and condensed and washed and collected for use as a fuel or otherwise. The remaining product is then agitated and washed with water from any suitable 40 supply, as a spray pipe, and allowed to settle, and is then washed with an alkaline material, from a suitable supply. The alkaline material is then removed, and the remaining product is washed with water

to remove any remaining alkaline material. 50 The remaining material is then reduced in the presence of steam or a suitable gas to produce the desired resulting lubricating oil above referred to.

In the accompanying drawings, I have 55 illustrated an apparatus suitable for the process, in which:

Figure 1 is a diagrammatic representation in sectional elevation, adapted to operate in the manner hereinafter set forth.

Fig. 2 is a longitudinal sectional view of the still, on the line II, II of Fig. 1.

I provide a cylindrical vessel 2 of suitable dimensions and capacity, in the center of which is a rotatable shaft 3 having a series 65 of agitating paddles or beaters 4. Shaft 3 is supported in a step box 5 having surrounding clearance for circulation and passes upwardly through a stuffing box 6 and a top bearing, and is rotated by gearing 70 7-8 and pulley 9, or other suitable means of vigorous agitation may be used. The vessel 2 is surrounded by a hot water or steam heating coil 10 by which the contents may be raised to any desired temperature under 75 control of the operator, and a valve 11 and conduit 12 provide for withdrawal of accumulated contents from the bottom of the vessel.

Petroleum distillate of proper quality and 80 containing a considerable percentage of unsaturated hydrocarbon may be first treated with sulfuric acid in the usual manner to remove any objectionable matter, and is then charged into vessel 2 through a man-hole 13. 85 Other treatment such as preliminary treatment with a small proportion of aluminum chlorid may be substituted for above acid treatment.

To this main body of petroleum distillate 90 I add a catalyst capable of polymerizing the unsaturated hydrocarbons present, as say about one-tenth of a pound, or less, of anhydrous aluminum chlorid or anhydrous hydrochloric acid or other halid per gallon 95 of distillate, or means for producing the same in a nascent condition. The catalyst may be introduced through manhole 13 or

through pipe 19. The vessel is then closed and the stirring paddles are actuated, operating to agitate the liquid upwardly, and the temperature is raised to a suitable degree, as from 300° to 400° F. However, the desired reaction will take place to some extent at ordinary temperatures, but slowly and incompletely, compared to the higher temperatures noted.

10 After stirring, for say an hour to an hour and one half, the stirring is stopped, and a heavy dark colored sludge, resulting from the operations, is allowed to settle into the bottom of vessel 2 and is drawn off through 15 valve 11.

Any light naphtha vapor in the vessel, *i. e.*, saturated hydrocarbons not exceeding say 5% to 10% of the total charge, may be drawn off through valve-controlled conduit

20 14 to condensing coil 15 and is condensed to a liquid. This product has an acid reaction and may be easily neutralized with soda. It is passed through a washer 16 to remove excess of soda and then drawn off 25 by outlet 17 and used as a fuel for engines, or as desired.

Such separate treatment of any portion of the main charge may, however, be omitted, and included in the general operation following.

The contents of agitating vessel 2 are cooled and again stirred, or otherwise agitated, and are then allowed to stand, when coloring substances will settle to the bottom 35 of the agitator and be drawn off. Cooling of the contents of vessel 2 may be effected by shutting off the steam or hot water supply to the coil 10 by valve 24 and opening valve 25 of a branch cold water supply pipe 26. 40 Soda or caustic soda solution is added by branch pipe 19<sup>a</sup>. The contents of agitating vessel 2 are again stirred and allowed to settle to the bottom. Excess of alkaline material is washed out with water from spray 45 pipe 19 and is drawn off from the bottom of agitator.

At this stage in the process, the remaining product will have become clear and of a light amber color, and is drawn off through 50 valve-controlled conduit 18 to still 20.

Still 20, into which the washed product is charged, is suitably mounted for operation over a furnace setting of common construction, and in which it is reduced by heat 55 action, in connection with steam or a suitable gas, introduced in the bottom of the still by pipe coil 21 having outlet perforations, of well known construction.

At first a certain proportion of naphtha 60 vapor is produced which passes by conduit 22 to condenser 23, and is drawn off and treated as above described to produce a liquid condensate. If all of the distillates from still 20 having a flash point higher 65 than about 300° F. are mixed together, an

excellent light lubricating oil is obtained, of low viscosity. If desired, also, the product may be divided as taken off, into separate fractional quantities of lubricating distillates, thereby obtaining a number of oils 70 having different gravities and viscosities.

The distillate from this oil has a remarkably low cold test, -60° to -70° F., and will remain perfectly bright below those temperatures.

The oil remaining in the still will now have been reduced to the desired flash and viscosity and, if desired, may be filtered through any suitable medium, as clay, bone, etc., to remove any suspended sediment, and 80 further improve the color and clarity. The natural color of the resulting oil when properly prepared being amber, very little filtering is required.

The oil resulting from the foregoing treatment, which may be conveniently divided into an oil having a flash point of approximately 300° F., and the heavier remaining oil, has the following desirable and interesting characteristics.

Although the stock of raw material from which the unsaturated hydrocarbons were obtained may have been obtained from paraffin base oils, such as distillate from Pennsylvania crude, the oil does not have the 90 usual properties of paraffin base lubricating oils, but has the properties of lubricating oils made from the finest asphaltic base crudes. The oil may be reduced so as to have a very high viscosity and at the same 95 time has a low specific gravity and a very low cold test. Thus, this very viscous oil will pour freely at a temperature at or much lower than zero, depending upon the viscosity to which the product is reduced, and at 100 the temperature of pouring and even much lower will remain perfectly bright. That is to say, it shows no separation of solid matter.

The oil of the flash point of approximately 300° F., constitutes substantially one-third 110 of the entire lubricating product. It is particularly adapted to use as an airplane machine gun oil or ice machine oil. This oil has a viscosity of 73 at 100° F., together with a flash test of 300° F., a fire test of 325° F., 115 and a cold test of approximately -60° F.

The heavier, or reduced, oil has a viscosity of 76 at 212° F., together with a flash test at this viscosity of 425° to 450° F., a fire test of from 460° to 480° F., and a cold test of 120 approximately -4° F. This oil is the grade which is of the greater importance and which is well adapted for use in internal combustion engines.

For purposes of comparison, the flash 125 point and cold test of oils of ordinary production which have corresponding viscosities may be given.

Thus a paraffin base oil having a viscosity of 73 at 100° F., has a flash point of 300° 130

F., but a cold test of approximately +30° F. An asphalt base oil having a viscosity of 73 at 100° F., will have a flash point of approximately 280° F., and a cold test of approximately -10° F.

Also a paraffin base oil having a viscosity of 76 at 212° F., will have a flash point of from 425° to 450° F., but will have a cold test of from +30° to +40° F. An asphalt 10 base oil having a viscosity of 76 at 212° F., will have a flash point of 375° to 390° F., and a cold test of +10° F.

All viscosities given are taken on the Saybolt universal viscosimeter.

15 The cuts above described are arbitrary and a number of cuts may be made to give oils of varying viscosity and accompanying characteristics. The grades above mentioned, however, clearly illustrate those desired characteristics of the entire bulk of lubricant; 20 namely, that it has a much lower cold test than a paraffin base oil of equal viscosity, and that it has a higher flash test and lower cold test than an asphalt base oil of equal 25 viscosity.

Either of the cuts described is suitable for use in shock absorbers, as they tend to obviate the necessity for changing the oil in the shock absorbers in accommodation to varying 30 temperatures. In other words, this oil has a lower coefficient of viscosity than the usual oils.

A further important characteristic of all 35 cuts of the lubricating oil, is the low carbon residue obtained by Conradson test. In the case of the cut having a viscosity of 73 at 100° F., the carbon residue by this test is merely a trace. In the case of the heavier reduced oil, having a viscosity of 76 at 212° 40 F., the carbon residue by Conradson test is less than 0.3 of one per cent. As this oil is adapted for use in internal combustion engines, and particularly in airplane engines in which the sparking points must be kept 45 clean, this feature is of great importance.

It should be noted that the lowest residue of an asphalt base oil by Conradson test is from 0.5 of one per cent. to 0.7 of one per cent.; while a paraffin base oil shows a residue of 1.3 per cent. to 1.7 per cent. These 50 figures are taken of oils having a viscosity of approximately 76 at 212° F.

When distilled under a vacuum, 60% of this oil distills within the range of 70° C., 55 showing that it is much more uniform in composition than usual or ordinary oils.

What I claim is:

1. A lubricating oil of synthetic production having a high flash point and low cold 60 test in relation to its viscosity; such relations being indicated by a flash of 425° Farenheit to 450° Farenheit and a cold test of approximately -4° Farenheit for a cut having a viscosity of 76 at 212° Farenheit.

2. A lubricating oil of synthetic production having a viscosity of 76 at 212° Farenheit, such oil having the characteristic that 60 per cent. thereof will distil within a range of 70° centigrade.

3. A lubricating oil of synthetic production characterized by having for a cut with a viscosity of 76 at 212° Farenheit, a carbon residue by Conradson test of less than 0.3 of one per cent.

4. A lubricating oil of synthetic production characterized by having for a viscosity of 76 at 212° Farenheit a carbon residue by Conradson test of less than 0.3 of one per cent.; said oil having the further characteristic that 60 per cent. of the body thereof having a viscosity of 76 at 212° Farenheit will distil within a range of 70° centigrade.

5. A lubricating oil of synthetic production having a high flash point and low cold 85 test in relation to its viscosity; such relations being indicated by a flash test of 425° Farenheit to 450° Farenheit and a cold test of approximately -4° Farenheit for a cut having a viscosity of 76 at 212° Farenheit; such oil having the added characteristic that 60 per cent. of the body thereof, having a viscosity of 76 at 212° Farenheit, will distil within a range of 70° centigrade.

6. A lubricating oil of synthetic production having a high flash point and low cold 95 test in relation to its viscosity; such relation being indicated by a flash test of 425° Farenheit and a cold test of approximately -4° Farenheit for a cut having a viscosity 100 of 76 at 212° Farenheit; such oil having the further characteristic that any cut throughout the body thereof has a carbon residue by Conradson test of less than 0.3 of one per cent.

7. A lubricating oil of synthetic production having a high flash point and low cold 105 test with relation to its viscosity; such relations being indicated by a flash point of 300° Farenheit and cold test of approximately -60° Farenheit for a cut having a viscosity of 73 at 100° Farenheit and a flash point of 425° to 450° Farenheit with a cold test of approximately -4° Farenheit for a body having a viscosity of 76 at 212° Farenheit.

8. A synthetically produced hydrocarbon oil corresponding generally to a crude oil of natural occurrence; such oil presenting throughout its body the characteristic of a 110 cold test varying with different cuts from thirty degrees Farenheit to ninety degrees Farenheit lower than that of a paraffin base crude of equal viscosity, and varying with different cuts from ten degrees Farenheit 115 to sixty degrees Farenheit lower than an asphalt base crude of equal viscosity.

9. A synthetically produced hydrocarbon oil corresponding generally to a crude oil of natural occurrence; such oil presenting 120

throughout its body the characteristic of a cold test varying with different cuts from thirty degrees Fahrenheit to ninety degrees Fahrenheit lower than that of a paraffin 5 base crude of equal viscosity, and varying with different cuts from ten degrees Fahrenheit to sixty degrees Fahrenheit lower than

an asphalt base crude of equal viscosity; said oil showing throughout a carbon residue by Conradson test of less than 0.3 of one 10 per cent.

In testimony whereof I hereunto affix my signature.

ROY H. BROWNLEE.